

May 13, 1930.

H. C. RENTSCHLER

1,757,976

VACUUM DEVICE AND METHOD OF MANUFACTURE

Filed Sept. 27, 1924



INVENTOR  
HARVEY C. RENTSCHLER.  
BY *M. F. Reger*  
ATTORNEY

## UNITED STATES PATENT OFFICE

HARVEY CLAYTON RENTSCHLER, OF EAST ORANGE, NEW JERSEY, ASSIGNOR TO  
WESTINGHOUSE LAMP COMPANY, A CORPORATION OF PENNSYLVANIA

## VACUUM DEVICE AND METHOD OF MANUFACTURE

Application filed September 27, 1924. Serial No. 740,409.

This application is a continuation-in-part of the copending application of Marden and Rentschler, Serial No. 679,489, filed December 8, 1923, clean-up and activation by misch metal and the rare earth metals, and assigned to the Westinghouse Lamp Company.

5 This invention relates to vacuum devices and more particularly to those utilizing a metallic clean-up agent, such as misch metal or the like.

10 In electron devices of the prior art, it has been common to employ a refractory metal such as molybdenum as an electrode material. Such material has the disadvantage that it is 15 expensive and rather difficult to work.

To overcome these difficulties, nickel has been substituted for a more refractory electrode material. However, metallic clean-up agents, such as misch metal or the like, upon 20 volatilization, attack the nickel when the latter is used as a carrier for agents of this character.

I have discovered that nickel as electrode 25 material may be replaced by iron, and that the latter is not deleteriously affected when the same functions as a carrier for a metallic clean-up agent upon volatilization thereof.

It is therefore an object of my invention to utilize iron as a carrier for a metallic clean-up agent embodied in evacuated electrical devices such as radio tubes, incandescent electric lamps and the like.

A more specific object of my invention is the use of iron as a plate material in radio 35 tubes and the like, whereby certain metallic clean-up agents, such as misch metal, may be secured thereto without the danger of causing injury or destruction thereto during the cleaning-up process, effected by heating or 40 volatilization of the clean-up agent.

A further object of my invention is the manufacture of radio tubes with plates, preferably constructed of relatively pure iron, 45 making use of misch metal as a clean-up material in the device, whereby the necessity for a C battery is dispensed with, as with such a tube the grid current starts when the grid potential is positive, rather than when it is 50 zero or negative, as usual in the case with

more strongly electropositive clean-up agents, such as magnesium.

Other objects and advantages of the invention will be apparent as the description proceeds.

In making an electron tube embodying my invention, no change is necessary in the manufacture thereof, other than substituting a plate of iron for one of nickel. It has been found that, contrary to what might be supposed, no alloying results when the iron plate with misch metal or rare earth metal applied thereon in the usual manner, is heated to cause vaporization of the misch metal. I preferably use the best grade of Norway iron to avoid introducing impurities into the bulb. In a number of tests, the heating was continued even after the misch metal was flashed sufficiently to clean-up the gases, in order to determine whether it was possible that such metal, at a still higher temperature, would attack the iron. In no case, however, did misch metal melt through the iron, as it did in similar instances with nickel. By the use of iron, I am enabled to make cheaper and yet better tubes.

An advantage of misch metal, not secured by a usual material, such as magnesium, is that the grid current does not start in the tube until the potential of the grid is positive, as contradistinguished from the negative or zero potential at which the grid current starts when using magnesium or other more strongly electro-positive metal. As an illustration, ten tubes of the 201-A type with misch metal clean-up material had a value of the grid potential at which the grid current started, varying from .3 to 1.1 volts positive. The average was .62 volts positive.

With a regular magnesium clean-up, the grid potential varied from -.4 to +.1 with an average of -.1. It will be apparent, therefore, that in using misch metal according to my invention, a C battery becomes unnecessary and one element in radio apparatus is, therefore, dispensed with.

A possible explanation of the reason for this desirable effect is that, if any misch metal is deposited on the grid during the activation thereof, it does not of itself, cause any grid

55

60

65

70

75

80

85

90

95

100

current to start until the grid is made positive from an external source. In other words, the deposition of misch metal, upon a grid formed of electronegative material such as molybdenum, does not appreciably affect its 5 operating characteristics, whereas, on the contrary, if the clean-up agent is magnesium, calcium, sodium or some other more strongly electropositive metal, when the same becomes 10 deposited on the grid, it so changes its operating characteristics that a grid current flows thereto because of its inherently positive surface, even though its potential from an outside source is zero or negative. Although 15 this is advanced as a plausible explanation, I do not wish to be limited thereto, as the result stated is secured regardless of how it is effected.

In order that the invention may be more 20 fully understood reference may be had to the accompanying drawing in which the single figure discloses a three electrode electron discharge device embodying my invention.

In this view, envelope 1 containing a filamentary cathode 2, grid or control electrode 3 and anode 4 is shown. A quantity 5 of misch metal or other metal of the cerium group of rare earth metals is secured to the anode 4 in any convenient manner. The anode 30 is formed of iron which is stable with respect to the getter 5 and which permits the getter to be vaporized therefrom without causing injury or destruction thereto. Upon vaporization, a portion of the misch metal is 35 vaporized onto the grid and gives a negative bias so that the grid current does not start until the grid is made positive from an external source.

Although I have described my invention 40 particularly with reference to radio tubes and other electron devices, it is to be understood that I contemplate using misch metal and the like for cleaning up residual gases in other evacuated devices, for example, incandescent 45 electric lamps, by applying the same to a carrier formed of iron and heating said carrier in the evacuated device to vaporize or sufficiently heat the same to effect the desired clean-up action.

50 The expression "rare earth metal of the cerium group" is used herein to designate in accordance with accepted classification, cerium, lanthanum, praseodymium, neodymium and samarium.

55 Although I have described what is now considered a preferred embodiment of my invention, it is to be understood that the same is merely illustrative and that other modifications may occur to those skilled in the art 60 within the spirit and scope of the appended claims.

What is claimed is:

1. An evacuated container having therein 65 a rare earth metal of the cerium group and a metallic member to which said rare earth

metal is attached, said metallic member being adapted to be heated to a sufficiently high temperature to vaporize said rare earth metal and being composed of iron with which said rare earth metal does not deleteriously react 70 during such vaporization.

2. An evacuated container having therein a quantity of misch metal and a metallic member to which said misch metal is attached, said metallic member being adapted 75 to be heated to a sufficiently high temperature to vaporize said misch metal and being composed of iron with which said misch metal does not deleteriously react during such vaporization.

3. An electrode for a vacuum device having a quantity of misch metal attached thereto, said electrode being composed of iron.

In testimony whereof, I have hereunto subscribed my name this 25th day of September, 1924.

HARVEY CLAYTON RENTSCHLER.

90

95

100

105

110

115

120

125

130